

## UNITED STATES PATENT OFFICE.

CARL D. HOCKER, OF EAST ORANGE, NEW JERSEY, ASSIGNOR TO WESTERN ELECTRIC COMPANY, INCORPORATED, OF NEW YORK, N. Y., A CORPORATION OF NEW YORK.

## COATING COMPOSITIONS.

No Drawing. Application filed December 18, 1923. Serial No. 680,343.

This invention relates to coating compositions, and its object is to produce a liquid coating composition which may be readily applied to an article and baked thereon to form a hard, tough, flexible and durable coating.

In particular it is desired to produce a liquid coating composition which is of such nature that it may be rapidly baked on a metallic article such as an electrical conductor to form a hard enamel which is flexible and inert to solvents, and which has good insulating properties.

In accordance with the general features of the invention, polymerized vegetable oil is used as the basis of a liquid coating composition. The vegetable oils which have been found most suitable are those such as tung oil and castor oil which have the properties of polymerizing and thereafter gelatinizing when heated. Such oils give the best results when polymerized to a state just short of gelatinization. To realize this state of polymerization, the oil may be heated in the presence of some substance, such as rosin oil, which will delay or prevent its gelatinization, as set forth in my copending application, Serial No. 633,322, filed April 19, 1923. Vegetable oils prepared in this way may be spread upon a metallic article and baked thereon to form a hard, flexible insulating enamel. Inasmuch as a liquid coating composition prepared from vegetable oils alone is slow baking the polymerized oil is mixed with certain substances which will decrease the time required to bake it on a metallic article, and which will for this reason considerably reduce the cost of coating such articles. The substances which have been found most satisfactory for this purpose are certain resin glycerides.

A resin such as Congo copal might be used; but it has been found preferable to use the glyceride of such a resin, both because it may be transformed by heat into a hard substance at a temperature similar to that at which vegetable oils are thus transformed, and because the glycerol converts the acid bodies of the resin into substances which are more inert chemically. As

such glycerides have a tendency when heat treated to gelatinize in the same manner that certain vegetable oils gelatinize, it is desirable to add during the esterification of the resin a substance such as rosin oil which will maintain the glycerides in an ungelatinized, liquid condition.

One feature of the invention consists in producing a liquid coating composition which contains a minimum amount of acid bodies likely to attack the metallic article during the baking to form metallic soaps. The presence of these soaps tends to make the coating less flexible when heated to a degree at which it has the necessary inertness to solvents.

After the addition of the glyceride, the mixture should be heated over a period of time, and solvents, added, if necessary, in order that the resulting composition will produce a smooth coating when applied to and baked on the metallic article. The composition is then spread on the metallic article and baked.

Such a composition bakes rapidly at a temperature similar to that at which vegetable oil hardens, and forms an enamel which is hard enough to withstand the treatment to which electrical conductors are normally subjected, which has a toughness greater than that of an enamel formed from vegetable oil alone, which is so flexible that a wire coated therewith may be sharply bent without cracking the enamel, and which has good insulating properties. Furthermore, this enamel is very resistant to the solvent action of the benzol or carbon tetrachloride contained in cleaning fluids commonly used upon enameled conductors of the linseed oil in certain varnishes with which enameled conductors are often coated, of the denatured alcohol used in shellacs, of the resin-rosin oil combinations or the paraffin used in the melted moisture-proofing compositions with which coils of enameled wire are often impregnated, or of the gasoline or benzene contained in various liquids which are likely to come in contact with enameled conductors.

Certain examples illustrating the above

processes are given below to enable the invention to be more readily practiced. When proportions are given they are by weight unless otherwise stated.

5 Tung oil (Chinese wood oil) is treated in any of the following ways:

(a) Equal parts of tung oil and rosin oil are mixed and the mixture heated at a temperature between 210° C. and 220° C. for 10 about two hours.

A glyceride of Congo copal is formed in any of the following ways:

(a') Two or more parts of rosin oil (preferably having a high boiling point) 15 are added to one part of Congo copal and the mixture heated at between 275° C. and 300° C. for two hours or until the copal is entirely fused. One gallon of glycerol for each fourteen pounds of Congo copal is then 20 added to the mixture and the temperature maintained at between 280° C. and 300° C. for about one hour. At the completion of this heating, the mass will still contain a considerable amount of uncombined copal 25 and the above treatment with glycerol is repeated until the acid number of the mixture is reduced to about 10. If apparatus is used which will prevent to a certain extent the volatilization of the glycerol, all the 30 glycerol may be added at once. During the treatment with glycerol the proportions of rosin oil to the copal should be maintained at not less than two to one.

(b') Congo copal is fused until it has lost 35 twenty percent to thirty-five percent of its weight. To one part of this fused copal is added two parts of rosin oil. Glycerol is then added, and the process continued in either of the ways indicated in (a') above.

(c') Congo copal is fused with an equal proportion of rosin, the resultant product heated with glycerol, preferably in the presence of rosin oil and the process continued as in (a') above.

(d') Three parts of Congo copal are fused as described in my Patent 1,422,861 of July 18, 1922, with two parts of those fatty acids derived from tung oil by saponification. Sufficient glycerol to neutralize 50 both the resin and the fatty acid is then added and the mixture heated, preferably in the presence of rosin oil, in the manner described in (a') above. A certain amount of tung oil is formed from the glycerol and 55 the tung oil fatty acids and is polymerized by the heating.

The tung oil prepared as in (a), above is then mixed with the resin glyceride as in one of the foregoing examples in approximately the following proportions:

Four parts of treated tung oil to one part of resin glyceride prepared as in (a'), (b'), or (c');

Three parts of treated tung oil to one

part of the mixture of resin glyceride and polymerized tung oil prepared as in (d');

The resulting mixture is heated for about six hours, when a suitable proportion of volatile solvent such as benzine or Hi-flash-naphtha is added. This composition is applied to the article to be coated and is baked thereon at or about a temperature of about 300° C. to drive off the benzene or naphtha, any excess of glycerol, and the rosin oil, and to harden the coating. If a thicker coating is desired, the application and baking of the composition may be repeated as many times as necessary.

Any substance which will perform a like function should be considered as the equivalent of any of the substances mentioned in the specific examples described above.

Castor oil, corn oil, soya bean oil, rape-seed oil, sesame oil, cottonseed oil and peanut oil, for instance, may be used in place of either the tung oil or the linseed oil and either of these two oils may replace the other. Other resin oils may be used in place of the rosin oil.

Manila copal and shellac are examples of other resins which will form gelatinizable esters with glycerol and are best adapted for use in this invention.

The term "gelatinization" as used herein is intended to describe the sudden thickening that occurs when vegetable oils or resin glycerides are polymerized beyond a certain degree by heat, as contrasted with the very gradual thickening which occurs during the preceding polymerization.

What is claimed is:

1. The process of forming an insulating enamel which comprises heating gelatinizable vegetable oil in the presence of a substance which will delay the gelatinization thereof, heating together a resin, resin oil and glycerol mixing the products so formed, heating the resulting mass and diluting the mass with a volatile material.

2. The process of forming a liquid coating composition which comprises heating tung oil with a mixture of glycerol and resin oil, heating glycerol with a mixture of Congo copal and resin oil, mixing the products so formed and heating the mixture.

3. The process of producing a liquid coating composition which comprises heating a mixture of tung oil and resin oil with a quantity of glycerol less than said tung oil and mixing therewith a resin glyceride.

4. The process of forming a liquid coating composition which comprises heating a mixture of resin oil and gelatinizable vegetable oil, mixing therewith a substance to give a quick baking quality to said coating composition, and heating the mixture.

5. The process of forming a liquid coating composition which comprises neutraliz-

ing the acid bodies of a substance having a quick baking quality with glycerol, heating a mixture of gelatinizable vegetable oil and resin oil, mixing the product so formed, and heating the resulting mixture.

6. The process of producing a liquid coating composition which comprises heating resin and resin oil, adding thereto sufficient glycerol to produce a glycerol ester of said

resin having a low acid number, and heating the resulting mixture, heating gelatinizable vegetable oil in the presence of resin oil, mixing the product so formed, and heating the resulting mass.

In witness whereof, I hereunto subscribe my name this 11 day of December, A. D. 1923.

CARL D. HOCKER.